



US006573034B2

(12) **United States Patent**  
Murabayashi

(10) **Patent No.:** US 6,573,034 B2  
(45) **Date of Patent:** Jun. 3, 2003

(54) **METHOD OF RESTORING BLACK-AND-WHITE PICTURE UNDER AGING PHENOMENA**

(75) Inventor: **Takao Murabayashi**, Tokyo (JP)

(73) Assignee: **Photo Murabayashi Ltd.**, Tokyo (JP)

(\*) Notice: Subject to any disclaimer, the term of this patent is extended or adjusted under 35 U.S.C. 154(b) by 8 days.

(21) Appl. No.: **09/769,937**

(22) Filed: **Jan. 25, 2001**

(65) **Prior Publication Data**

US 2002/0098450 A1 Jul. 25, 2002

(51) **Int. Cl. 7** ..... **G03C 5/26**

(52) **U.S. Cl.** ..... **430/401**

(58) **Field of Search** ..... 430/401

(56) **References Cited**

U.S. PATENT DOCUMENTS

4,323,974 A \* 4/1982 Sekigawa ..... 382/272  
4,356,555 A \* 10/1982 Ejiri et al. ..... 382/254

\* cited by examiner

*Primary Examiner*—Hoa Van Le

(74) *Attorney, Agent, or Firm*—Jordan and Hamburg LLP

(57) **ABSTRACT**

Method of restoring black-and-white picture under aging phenomena includes ethylene alcohol wipe process proceeded to wipe a surface of photograph dry plate or negative film taken the black-and-white picture and preserved for a long term by ethylene alcohol and allow it to dry; silver mirror removal process proceeded to wipe and drop a silver part on the surface of image of the photograph dry plate or negative film by silver mirror removal liquid after the ethylene alcohol wipe process is proceeded; and tail end process proceeded such that the photograph dry plate or negative film removed the silver mirror in the removal process is washed in dear water by water or stream and it can be dried. Accordingly, the silver mirror part on the surface of the image on the photograph dry plate or negative film of the black-and-white picture under aging phenomena is removed, or a metallic uniting silver is disarranged, and the silver mirror part can be replaced with silver which makes original black, so that it is possible to restore it to the photograph dry plate or negative film that obtains an original black-and-white picture.

**2 Claims, 13 Drawing Sheets**



**FIG. 1**

FIG. 2



FIG. 3



FIG. 4



FIG.5



FIG. 6



FIG. 7



FIG. 8



FIG. 9



FIG. 10



**FIG. 11****FIG. 12**

FIG. 13



**FIG. 14****FIG. 15**

FIG. 16



FIG. 17



**METHOD OF RESTORING BLACK-AND-WHITE PICTURE UNDER AGING PHENOMENA**

**BACKGROUND OF THE INVENTION**

The present invention relates generally to a method of restoring the black-and-white picture under aging phenomena, the method restoring the aging phenomena such as silver mirror ("Gin Kabun" in Japanese), discoloration or the like of the photograph dry plate, negative film or black-and-white picture which is taken a picture of the black-and-white and is preserved for a long term.

In the conventional photograph dry plate, negative film or black-and-white picture taken the black-and-white picture, silver formed the image comes to shoot metallic luster on the surface of the image and it changes to the silver mirror by the preservation of a long term so far, and the silver mirror appears remarkably in the shade part of the image. Accordingly, the decrease in the picture quality is invited, and there is a fault of ruining original consideration to which the photograph is involved and the meaning

**SUMMARY OF THE INVENTION**

Accordingly, it is an object of the present invention to provide the method of restoring the black-and-white picture under aging phenomena that can be made an original black-and-white picture, photograph dry plate or negative film with silver which makes original in the silver part black by disarranging a metallic uniting the removal or silver and replacing the silver part on the surface of the image of the black-and-white picture changed.

The novel features which are believed to be characteristic of the invention, both as to its organization and method of operation, together with further objects and advantages thereof, are described below with reference to the accompanying drawings in which a presently preferred embodiment of the invention is illustrated as an example.

It is to be expressly understood, however, that the drawings are for the purpose of illustration and description only and are not intended as a definition of the limits of the invention.

**BRIEF DESCRIPTION OF THE DRAWINGS**

FIG. 1 is a view of a process showing a first embodiment of the present invention;

FIG. 2 is an explanation view of a process for wiping by ethylene alcohol;

FIG. 3 is an explanation view of a process for removing silver mirror;

FIG. 4 is an explanation view of a tail end process;

FIG. 5 is a view of a process showing a second embodiment of the present invention;

FIG. 6 is an explanation view of a preprocessing process;

FIG. 7 is an explanation view of a process for spreading hardener;

FIG. 8 is an explanation view of a process for removing hardener;

FIG. 9 is an explanation view of a process for bleaching;

FIG. 10 is an explanation view of a process for removing bleacher;

FIG. 11 is an explanation view of process for exposing;

FIG. 12 is an explanation view of process for developing;

FIG. 13 is an explanation view of a fixation process;

FIG. 14 is an explanation view of a process for removing hypo;

FIG. 15 is an explanation view of a tail end process;

FIG. 16 is a view of a process showing a third embodiment of the present invention; and

FIG. 17 is an explanation view of a tail end process.

**DETAILED DESCRIPTION**

Preferred embodiments of the present invention are described in more detail below referring to the accompanying drawings.

An understanding of the present invention may be best gained by reference FIGS. 1 to 4. FIGS. 1 to 4 illustrates the method of restoring the black-and-white picture under aging phenomena of a first embodiment of the present invention. The numeral 1 is a method of restoring the black-and-white picture under aging phenomena of this invention. The above restoring method 1 is composed of ethylene alcohol wipe process 3, silver mirror removal process 5, and tail end process 6.

The ethylene alcohol wipe process 3 is proceeded to wipe the surface of photograph dry plate or negative film 2 which are taken a picture of the black-and-white picture and preserved for a long term by ethylene alcohol 3a and allow it to dry. After the ethylene alcohol wipe process 3 is proceeded, the silver mirror removal process 5 is proceeded to wipe and drop the silver part 4 of the surface of the image of the photograph dry plate or negative film 2A by the silver mirror removal liquid 5a.

After the silver mirror removal process 5 is proceeded, the tail end process 6 is proceeded such that the photograph dry plate or negative film 2B which removed the silver mirror of the removal process 5 is washed in clear water by water or stream 6a and it can be dried.

In the ethylene alcohol wipe process 3, the dirt of the surface of the photograph dry plate or negative film 2 is washed by the wipe material 7 such as cotton, cloths including absorbent cloths to contain ethylene alcohol 3a enough. Then it dries the ethylene alcohol that adheres to the photograph dry plate or negative film 2 with natural seasoning or a heater, etc.

In the silver mirror removal process 5, the wipe material 7A such as cotton and cloths including the absorbent cloths contains a small amount of the silver mirror removal liquid 5a. The silver mirror part 4 is wiped until the silver mirror can be removed and dropped.

The silver mirror removal liquid 5a used in the silver mirror removal process 5 is a mixture—one to ten part methanol and one part solution of salt of 0.5 to 25 percent.

The tail end process 6 is proceeded to remove the removal liquid 5a used in the above-mentioned removal process 5, the removal liquid 5a is dried by natural seasoning in the place without dust and where it is well ventilated after it washes in clear water to flush the silver mirror removal liquid 5a in stream 6a.

Other embodiments of the present invention will now be described referring to FIGS. 5 to 17. Through the drawings of the embodiments, like components are denoted by like numerals as of the first embodiment and will not be further explained in great detail.

A second embodiment of the present invention is shown in FIGS. 5 to 15. It is distinguished from the first embodiment by the fact that the restoring method 1 is replaced from

another method including a head end process **8**, process for spreading hardener **9**, process for removing hardener **10**, process for bleaching **11**, process for removing bleacher **12**, process for exposing **13**, process for developing **14**, fixation process **15**, process for removing hypo **16** and tail end process **6A**.

In the head end process **8**, water **8a** cleans up the surface of photograph dry plate or negative film **2** and this process **8** makes the surface thereof to contain water. The process **8** is proceeded in about two minutes.

After the head end process **8** is proceeded, the surface of photograph dry plate or negative film is spread hardener **9a** or the photograph dry plate or negative film itself dipped into the hardener **9a** in about eight minutes such that the gelatin of the photograph dry plate or the image of the negative film **2C** is hardened in the hardener spreading process **9**.

After the gelatin of the image hardens in the hardener spreading process **9**, the hardener **9a** is removed from photograph dry plate or negative film **2D** by washing in clear water about ten minutes in the hardener removal process **10**.

After the hardener removal process **10** is proceeded, the silver compound in discoloring discoloration of the image and silver mirror part are bleached at bleacher **11a** in the bleaching process **11** about two to five minutes.

In the bleacher removal process **12**, the bleacher **11a** is removed by washing in clear water about three minutes, and the cleaning solution **12a** washes in clear water for about thirty minutes, after the bleacher **11a** which remains in the image part which cannot be removed by the washing in clear water is decomposed by cleaning solution **12a** about five minutes.

In the exposing process **13**, the halogenated silver produced in the bleaching part according to the bleacher removal process **12** is exposed at the state that light is applied and exposed enough.

After that, it develops with develop solution **14a** used in general in the development process **14** at about two to three minutes.

In the fixation process **15**, after the development process **14** is proceeded, the exposed negative film soaks to stop solution **15a** for about thirty seconds, the develop solution **14a** is neutralized, and halogenated silver which remains on the photograph dry plate or negative film is decomposed for about five minutes by fixing solution **15b**. After that, the fixing solution **15b** is removed by washing in clear water for about three minutes.

After the fixation process **15** is proceeded, hypo ("hypo" means for sodium thiosulfate) which remained on photograph dry plate or negative film **2E** is decomposed and removed by hypo removal liquid **16a** at about six minutes in the hypo removal process **16**.

After that, in the tail end process **6A**, after the compound that remains on the photograph dry plate or negative film is removed almost completely by washing in clear water for about thirty minutes or more and it dries generally or naturally.

A restoring method according to the second embodiment may be proceeded.

In addition, the hardener **9a**, as used at 20° C., which is the liquid used by this restoring method in processing temperature is composed of sodium sulfite of fifty gram, glacial acetic acid of twenty milliliter, and potassium alum of fifty gram.

The bleacher **11a** is composed of A liquid which adds potassium permanganate of five gram to water of one liter,

B liquid which adds hydrochloric acid of 100 milliliter of thirty-five percent to the water of one liter at the same amount of the A liquid, and liquid making to mixture liquid of twenty liter which mixes three to thirty-eight times is added to hydrobromic acid of 0.2 to 2 milliliter.

Cleaning solution **12a** is potassium metabisulfite of one to ten percent.

Developer **14a** uses the one used in general.

Stop solution **15a** is the glacial acetic acid of three percent.

Fixing solution **15b** is the mixture that sodium thiosulfate (hypo) of 240 gram is added to the water of one liter.

Hypo removal liquid **16a** is sodium metasulfite of two percent.

A third embodiment of the present invention is shown in FIGS. **16** and **17**. It is distinguished from the second embodiment by the fact that the tail end process **6A** is replaced from with another method **6B**. In this method **6B**, a similar process of the second embodiment of the above-mentioned is done by using black-and-white picture **3**, the black-and-white picture **3A** which is naturally dry is placed between two flat pressurizing boards **17** and **17**, and it pressurizes with a weight **18** or the like and is flattened.

A restoring method with the tail end process **6B** according to the third embodiment may be proceeded.

As set forth above, the advantages of the invention are as follows:

(1) Method of restoring black-and-white picture under aging phenomena includes ethylene alcohol wipe process proceeded to wipe a surface of one of photograph dry plate and negative film which is taken the black-and-white picture and preserved for a long term by ethylene alcohol and allow it to dry; silver mirror removal process proceeded to wipe and drop a silver part on the surface of image of the photograph dry plate and the negative film by silver mirror removal liquid after the ethylene alcohol wipe process is proceeded; and tail end process proceeded such that one of the photograph dry plate and negative film which removed the silver mirror in the removal process is washed in dear water by water or stream and it can be dried. Accordingly, the silver mirror part on the surface of the image of the photograph dry plate and the negative film of the black-and-white picture under aging phenomena is removed, or a metallic uniting silver is disarranged, and the silver mirror part can be replaced with silver which makes original black.

Therefore, it is possible to restore it to the photograph dry plate and the negative film that obtains an original black-and-white picture.

(2) As discussed above, because it is possible to restore it to an original black-and-white picture in the ethyl alcohol wipe process, the silver mirror removal process, and the postprocessing process where dryness of washing in dear water is done, the work is easy comparing it, and it is possible to do in short course.

(3) Method of restoring black-and-white picture under aging phenomena includes head tail process proceeded that a surface of one of photograph dry plate, negative film and black-and-white picture is cleaned up by the water and it makes the surface thereof to contain water; process for spreading hardener proceeded that the hardener is spread on the surface of one of photograph dry plate, negative film and black-and-white picture or receives one of the photograph dry plate, negative film and black-and-white picture such that gelatin of one of the photograph dry plate and an image of the negative film is hardened after the head tail process is

proceeded; process for removing the hardener proceeded that after the gelatin of the image hardens in the hardener spreading process, the hardener is removed from one of the photograph dry plate and negative film by washing in dear water; process for bleaching proceeded that, silver compound in discoloring discoloration of the image and silver mirror part are bleached at a bleach solution after the hardener removal process is proceeded; process for removing the bleach solution proceeded that the bleach solution is removed by washing in dear water, and cleaning solution is removed by washing in dear water after the bleach solution which remains in the image part which cannot be removed by the washing in dear water is decomposed by the cleaning solution; process for exposing proceeded that halogenated silver which produced in the bleaching part according to the 15 bleach solution removal process is exposed at the state that light is applied enough; process for developing proceeded that develops with develop solution after the exposing process is proceeded; fixation process proceeded that the develop solution is neutralized by stop solution, and halogenated silver which remains on one of the photograph dry plate, negative film and black-and-white picture is decomposed by fixing solution, and after that, the fixing solution is removed by washing in clear water; process for removing 20 hypo proceeded that, hypo remained on one of the photograph dry plate, negative film and black-and-white picture is decomposed and removed by hypo removal liquid after the fixation process is proceeded; and tail end process proceeded that compound remains on one of the photograph dry plate, negative film and black-and-white picture is removed almost 25 completely by washing in clear water and then allowing to dry after the hypo removal process is proceeded, so that it is possible to replace it with silver which makes original black by removing the silver mirror part on the surface of the image of the photograph dry plate of the black-and-white 30 picture changed under aging phenomena, the negative film, and the black-and-white picture and the silver compounds. 35

Therefore, it is possible to restore it to the black-and-white picture, the photograph dry plate and the negative film that obtains an original black-and-white picture. 40

What is claimed is:

1. Method of restoring black-and-white picture under aging phenomena includes:

head tail process proceeded that a surface of one of photograph dry plate, negative film and black-and-white picture is cleaned up by the water and it makes the surface thereof to contain water; 45

process for spreading hardener proceeded that the hardener is spread on the surface of one of photograph dry plate, negative film and black-and-white picture or

receives one of the photograph dry plate, negative film and black-and-white picture such that gelatin of one of the photograph dry plate and an image of the negative film is hardened after the head tail process is proceeded;

process for removing the hardener proceeded that after the gelatin of the image hardens in the hardener spreading process, the hardener is removed from one of the photograph dry plate and negative film by washing in clear water;

process for bleaching proceeded that silver compound in discoloring discoloration of the image and silver mirror part are bleached at a bleach solution after the hardener removal process is proceeded;

process for removing the bleach solution proceeded that the bleach solution is removed by washing in dear water, and cleaning solution is removed by washing in clear water after the bleach solution which remains in the image part which cannot be removed by the washing in clear water is decomposed by the cleaning solution;

process for exposing proceeded that halogenated silver which produced in the bleaching part according to the bleach solution removal process is exposed at the state that light is applied enough;

process for developing proceeded that develops with develop solution after the exposing process is proceeded;

fixation process proceeded that the develop solution is neutralized by stop solution, and halogenated silver which remains on one of the photograph dry plate, negative film and black-and-white picture is decomposed by fixing solution, and after that, the fixing solution is removed by washing in clear water;

process for removing hypo proceeded that, hypo remained on one of the photograph dry plate, negative film and black-and-white picture is decomposed and removed by hypo removal liquid after the fixation process is proceeded; and

tail end process proceeded that compound remains on one of the photograph dry plate, negative film and black-and-white picture is removed almost completely by washing in clear water and then allowing to dry after the hypo removal process is proceeded.

2. The Method of restoring the black-and-white picture under aging phenomena according to claim 1, wherein the tail end process proceeds a natural seasoning.

\* \* \* \* \*